

## UNITED STATES PATENT OFFICE.

JOHN MURDOCH SKELLEY AND JAMES MERSON, OF BATTERSEA, LONDON, ENGLAND,  
ASSIGNORS TO CONTINUOUS REACTION COMPANY, LIMITED, OF LONDON, ENGLAND.

## MANUFACTURE OF FERROTUNGSTEN.

No Drawing.

Application filed May 29, 1922. Serial No. 564,615.

*To all whom it may concern:*

Be it known that we, JOHN MURDOCH SKELLEY and JAMES MERSON, both subjects of the King of Great Britain, residing at

5 155 Church Road, Battersea, London, England, have invented new and useful Improvements in the Manufacture of Ferrotungsten, of which the following is a specification.

10 This invention relates to improvements in the manufacture of ferrotungsten, i. e. alloys of tungsten and iron in various proportions, containing up to about 85 per cent of tungsten respectively.

15 These alloys have hitherto been manufactured as a rule from ores or mixtures containing iron and tungsten by reduction either in the electric furnace or by the alumino-thermic process. In some cases the

20 alumino-thermic reduction has been effected by means of a mixture of aluminium and ferrosilicon, but it has not been possible to dispense with the use of a substantial proportion of aluminium, which is a relatively costly reducing agent.

25 The present invention is based upon the discovery that if ores or mixtures containing iron and tungsten in the form of oxides be mixed with pulverized silicon or ferro-

30 silicon and a suitable oxidizing agent containing nitrogen such as sodium nitrate, but without aluminium, reaction may be initiated at a point in a cold or heated mixture as in the alumino-thermic process, and

35 if suitable proportions of the ingredients be used the reaction proceeds to completion, ferrotungsten practically free from carbon and silicon resulting.

According to this invention, therefore, 40 ferrotungsten is produced without the aid of aluminium by the silico-thermic reduction of a mixture of oxide of iron with oxide of tungsten, or of an ore containing iron and tungsten in the form of oxide, by means 45 of silicon or ferrosilicon in the presence of a suitable oxidizing agent containing nitrogen, such as sodium nitrate or calcium nitrate.

As a rule, the richer the reducing agent is 50 in silicon, the better is the reaction. Commercial silicon, which contains up to about 95% Si, or ferrosilicon containing from 90 to 70% Si, can be used with excellent results. It will be understood that with ferro-

silicon containing lower proportions of silicon the reaction becomes more sluggish and a limiting composition is reached which depends upon the method of working.

Commercial ores, with or without the addition of iron oxide, can be used for the purpose of the invention and are if necessary subjected to a preliminary treatment having for its object the removal of tin compounds, sulphur or other injurious matter such as arsenic or bismuth or an excess of silicious impurities, and conversion of all the iron and tungsten into the form of oxide.

The following example illustrates the invention:—

A commercial tungsten ore is subjected to a preliminary purification to remove any tin and other undesired constituents present and is then roasted till free from sulphur. Of the product, containing 70 per cent of  $WO_3$ , 16 per cent of  $FeO$  and 8 per cent of  $MnO$ , 100 lbs. are mixed with 20 $\frac{1}{4}$  lbs. of ferrosilicon (90% Si) and 5 lbs. of sodium nitrate. Preferably 5 lbs. of calcium fluoride are added to enhance the fluidity of the slag. The mixture is put into a crucible and reaction is initiated as in the alumino-thermic process.

What we claim is:—

1. The manufacture of ferrotungsten without the aid of aluminium by the silico-thermic reduction of iron oxide and tungsten oxide in the presence of an oxidizing agent containing nitrogen.

2. The manufacture of ferrotungsten without the aid of aluminium by the silico-thermic reduction of iron oxide and tungsten oxide in the presence of sodium nitrate.

3. The manufacture of ferrotungsten by purifying tungsten ore to remove any tin and other undesired constituents present, roasting the residue to remove sulphur, mixing with the product ferrosilicon and an oxidizing agent containing nitrogen, and producing reaction as in the well known alumino-thermic process.

4. The manufacture of ferrotungsten without the aid of aluminium by the silico-thermic reduction of iron oxide and tungsten oxide in the presence of a nitrate oxidizing agent.

5. The manufacture of ferrotungsten by purifying tungsten ore to remove any tin and other undesired constituents pres-

ent, roasting the residue to remove sulphur, mixing with the product ferrosilicon and a nitrate oxidizing agent, and producing reaction as in the well known alumino-thermic process.

6. The manufacture of ferrotungsten by a silico-thermic reaction in a mixture of 70 parts of tungsten oxide, 16 parts of iron

oxide, 8 parts of manganese oxide, 20 $\frac{1}{4}$  parts of ferrosilicon and 5 parts of sodium nitrate. 10

In testimony that we claim the foregoing as our invention we have signed our names this 17th day of May, 1922.

JOHN MURDOCH SKELLEY.  
JAMES MERSON.